

## UNITED STATES PATENT OFFICE

2,025,618

## DYEING LEATHER

Emil Senn, Riehen, near Basel, Switzerland, assignor to J. R. Geigy A. G., Basel, Switzerland, a firm

No Drawing. Application November 22, 1934, Serial No. 754,370. In Germany December 7, 1933

4 Claims. (Cl. 8—5)

This invention is an improvement in or modification of that described in the specification of a patent application Ser. No. 754,369 filed by the same inventor on the same day. That specification relates to the application of a certain group of amino-azobenzene-dyestuffs for dyeing leather, especially chrome leather, throughout.

According to the present invention, leather, especially chrome leather, can be through-dyed to a substantial degree or even completely by using instead of the dyestuffs used in the aforesaid specification amino-azobenzene sulphonic acids containing in the residue of the coupling component an amino-group substituted by a mono- or polyhydroxyalkyl group. Hitherto N-hydroxyalkylated acid azo-dyestuffs have been used only for dyeing textile fibres.

The yellow azo-dyestuffs hitherto used for dyeing leather, such as Orange II from diazotized sulphanic acid and  $\beta$ -naphthol (Schultz Farbstofftabellen, 6th edition, No. 139) or Metanil Yellow Extra from diazotized metanilic acid and diphenylamine (Schultz, No. 134) or the nitrated azo-dyestuff from diazo-sulphanilic acid and diphenylamine (Schultz, No. 141) are capable of dyeing chrome leather only superficially. In contrast thereto the dyestuffs used in accordance with the invention penetrate deeply into the leather and in most cases they dye it completely through. Leather, especially chrome leather, which has been dyed in accordance with the invention has great advantages. Its section is dyed throughout so that undyed portions are not exposed by damage to the surface or by wear during use.

Only a few dyestuffs which are capable of penetrating deeply into the interior of the hide or of dyeing chrome leather throughout have hitherto been known; for example, the yellow mono-azo-dyestuffs which are obtained from diazotized 2-chloro-4-amino-1-methylbenzene-6-sulphonic acid and resorcinol or a substitution product or homologue thereof dye chrome leather completely through. By the provision of a whole series of dyestuffs which are capable of penetrating into the interior of the leather without the addition of alkali and of dyeing it through to a substantial extent, the invention involves an important addition to the art of leather dyeing.

In carrying out the invention the leather may be dyed in accordance with the following procedure:

## Dyeing prescription

The neutralized hides are dyed in the cask with

150-200 per cent of water at a temperature of 65° C. The cask is set in motion and a solution of the dyestuff is introduced through the hollow axle of the cask. After 45 minutes the fat liquor is added and the cask is then kept in motion for a further 45 minutes. In the case of particularly heavy hides the duration of the dyeing must be suitably prolonged. In general a quantity of dyestuff amounting to 1-2 per cent of the weight of the material suffices for producing powerful through-dyeings.

The dyestuffs used in accordance with the invention may be made by the usual method, which is illustrated in the following examples. In these examples and in the table are described the production, composition and dyeing properties of a number of representatives of the group of dyestuffs of the amino-azobenzene series, but it will be understood that this does not exhaust all the possibilities within the scope of the invention.

In the following examples the parts are by weight:—

## Example 1

173 parts of 3-aminobenzene-1-sulphonic acid are diazotized in the usual manner and the diazo-solution is combined at 0-3° C. with 181 parts of dihydroxy-ethyl-aminobenzene which has previously been dissolved by means of the quantity of hydrochloric acid required to produce a solution which is faintly acid to Congo. The reaction is maintained faintly acid to Congo by addition of a solution of sodium acetate. When the formation of the dyestuff is finished the solution is made weakly alkaline by the addition of sodium carbonate, heated and the dyestuff precipitated by salting out. The dyestuff is a yellow crystalline powder which dyes leather, especially chrome leather, according to the foregoing prescription a powerful yellow throughout. The dyestuff of this example has the following formula:



## Example 2

127.5 parts of 2-chloro-1-aminobenzene are diazotized in the usual manner and the diazo-compound is coupled in a medium acid with acetic acid with 261 parts of 3-dihydroxy-ethylaminobenzene-1-sulphonic acid. When coupling is finished the dyestuff is isolated by salting out after the solution has been made alkaline with sodium carbonate. The dyestuff is a yellow powder which dyes chrome leather a powerful yellow both on

the surface and in the interior. The dyestuff of this example has the following formula:



Example 3

138 parts of 4-nitro-1-aminobenzene are diazotized and the diazo-solution is mixed with a solution of 225 parts of 3-N-ethylhydroxyethylaminobenzene-1-sulphonic acid. The coupling is carried to the end in a medium acid with acetic acid. The solution is then made alkaline by the addition of sodium carbonate and the dyestuff is precipitated by salting out in the form of a dark crystalline powder. It dyes chrome leather in powerful even brownish-red shades both on the surface and in the interior. The dyestuff of this example has the following formula:

20



Example 4

218 parts of 5-nitro-2-aminobenzene-1-sulphonic acid are diazotized with the required quantity of nitrite and hydrochloric acid and the diazo-compound is coupled with 215.5 parts of 3-chloro-1-dihydroxyethylaminobenzene in a solution which is faintly acid to Congo. By the addition of sodium acetate the reaction is maintained faintly acid to Congo throughout the coupling. When the formation of the dyestuff is finished the solution is rendered alkaline by the addition of sodium carbonate and the dyestuff is isolated in the usual manner. It is obtained in the form of a dark red powder which dyes chrome leather deep Bordeaux red shades on the surface and dark red-violet shades in the interior. The dyestuff of this example has the following formula:

5

10

15

20

25



Table

| 30 | Dyestuff.                                    |                                                                      | Dyeing on leather        |                          | 30                       |
|----|----------------------------------------------|----------------------------------------------------------------------|--------------------------|--------------------------|--------------------------|
|    | Diazo-component                              | Azo-component                                                        | On the surface           | In the interior          |                          |
| 1  | 2-chloro-1-aminobenzene                      | 3-dioxyethylamino-benzene-1-sulphonic acid                           | Powerful yellow          | Powerful yellow          | Powerful yellow          |
| 2  | 2,5-dichloro-1-aminobenzene                  | 3-dioxyethylamino-benzene-1-sulphonic acid                           | Deep orange              | Deep orange              | Deep orange              |
| 3  | 3,4-dichloro-1-aminobenzene                  | 3-dioxyethylamino-benzene-1-sulphonic acid                           | Powerful orange-yellow   | Powerful orange-yellow   | Powerful orange-yellow   |
| 4  | 2-nitro-1-aminobenzene                       | 3-dioxyethylamino-benzene-1-sulphonic acid                           | Brownish-orange          | Brownish-orange          | Powerful brownish orange |
| 5  | 3-nitro-1-aminobenzene                       | 3-dioxyethylamino-benzene-1-sulphonic acid                           | Orange-yellow            | Orange-yellow            | Orange-yellow            |
| 6  | 3-nitro-1-aminobenzene                       | 3-N-ethoxyethyl-aminobenzene-1-sulphonic acid                        | Powerful yellow          | Powerful yellow          | Powerful yellow          |
| 7  | 4-nitro-1-aminobenzene                       | 3-dioxyethylamino-benzene-1-sulphonic acid                           | Pale Bordeaux red        | Pale Bordeaux red        | Deep Bordeaux red        |
| 8  | 4-nitro-1-aminobenzene                       | 3-N-ethoxyethyl-aminobenzene-1-sulphonic acid                        | Powerful brownish-red    | Powerful brownish-red    | Powerful brownish-red    |
| 9  | 4-chloro-2-nitro-1-aminobenzene              | 3-dioxyethylamino-benzene-1-sulphonic acid                           | Brown-orange             | Brown-orange             | Powerful brown-orange    |
| 10 | 2,6-dichloro-4-nitro-1-aminobenzene          | 3-dioxyethylamino-benzene-1-sulphonic acid                           | Pale yellow-brown        | Pale yellow-brown        | Orange-brown             |
| 11 | 2,4-dinitro-1-aminobenzene                   | 3-dioxyethylamino-benzene-1-sulphonic acid                           | Red-violet               | Red-violet               | Deep red-violet          |
| 12 | 3-nitro-4-amino-1-methylbenzene              | 3-dioxyethylamino-benzene-1-sulphonic acid                           | Reddish-yellow           | Reddish-yellow           | Powerful reddish yellow  |
| 13 | 4-nitro-2-amino-1-methoxybenzene             | 3-dioxyethylamino-benzene-1-sulphonic acid                           | Brownish-orange          | Brownish-orange          | Powerful brownish-orange |
| 14 | 4-nitro-2-amino-1-oxyethylbenzene            | 3-dioxyethylamino-benzene-1-sulphonic acid                           | Brownish-orange          | Brownish-orange          | Brownish-orange          |
| 15 | 3-nitro-4-amino-1-ethoxybenzene              | 3-dioxyethylamino-benzene-1-sulphonic acid                           | Orange-brown             | Orange-brown             | Powerful orange-brown    |
| 16 | 6-nitro-3-amino-4-methoxy-1-methylbenzene    | 3-dioxyethylamino-benzene-1-sulphonic acid                           | Dark red-brown           | Dark red-brown           | Deep dark red-brown      |
| 17 | 3-aminobenzene-1-sulphonic acid              | Dioxyethylamino-benzene                                              | Pure yellow              | Pure yellow              | Powerful pure yellow     |
| 18 | 3-aminobenzene-1-sulphonic acid              | Di-( $\beta$ : $\gamma$ -dioxy)-propylaminobenzene                   | Yellow                   | Yellow                   | Yellow                   |
| 19 | 4-aminobenzene-1-sulphonic acid              | Dioxyethylamino-benzene                                              | Yellow                   | Powerful yellow          | Powerful yellow          |
| 20 | 4-aminobenzene-1-sulphonic acid              | Di-( $\beta$ : $\gamma$ -dioxy)-propylaminobenzene                   | Reddish-yellow           | Reddish-yellow           | Reddish-yellow           |
| 21 | 4-chloro-2-aminobenzene-1-sulphonic acid     | 3-dioxyethylamino-benzene-1-sulphonic acid                           | Reddish-yellow           | Reddish-yellow           | Reddish-yellow           |
| 22 | 6-chloro-3-aminobenzene-1-sulphonic acid     | Di-( $\beta$ : $\gamma$ -dioxy)-propylaminobenzene                   | Powerful reddish-yellow  | Powerful reddish-yellow  | Powerful reddish-yellow  |
| 23 | 2,5-dichloro-4-aminobenzene-1-sulphonic acid | 3-di-( $\beta$ : $\gamma$ -dioxy)-ethylaminobenzene-1-sulphonic acid | Pale brownish-orange     | Pale brownish-orange     | Orange-brown             |
| 24 | 2,5-dichloro-3-aminobenzene-1-sulphonic acid | 3-di-( $\beta$ : $\gamma$ -dioxy)-ethylaminobenzene-1-sulphonic acid | Brownish-orange          | Brownish-orange          | Brownish-orange          |
| 25 | 3-nitro-4-aminobenzene-1-sulphonic acid      | Di-( $\beta$ : $\gamma$ -dioxy)-propylaminobenzene                   | Brown-orange             | Brown-orange             | Powerful brown-orange    |
| 26 | 4-nitro-2-aminobenzene-1-sulphonic acid      | 3-N-ethoxyethylamino-benzene-1-sulphonic acid                        | Brownish-yellow          | Brownish-yellow          | Powerful brownish yellow |
| 27 | 4-nitro-2-aminobenzene-1-sulphonic acid      | Oxyethylamino-benzene                                                | Dull yellow              | Dull yellow              | Brownish yellow          |
| 28 | 4-nitro-2-aminobenzene-1-sulphonic acid      | 3-oxyethylamino-1-methylbenzene                                      | Brown-yellow             | Brown-yellow             | Powerful brown-orange    |
| 29 | 4-nitro-2-aminobenzene-1-sulphonic acid      | 3-dioxyethylamino-1-methylbenzene                                    | Orange-brown             | Orange-brown             | Deep orange-brown        |
| 30 | 4-nitro-2-aminobenzene-1-sulphonic acid      | 4-chloro-2-dioxyethylamino-1-methoxybenzene                          | Brown-yellow             | Brown-yellow             | Brown-yellow             |
| 31 | 4-nitro-2-aminobenzene-1-sulphonic acid      | 3-dioxyethylamino-1-oxybenzene                                       | Powerful brownish-yellow | Powerful brownish yellow | Powerful brownish yellow |
| 32 | 5-nitro-2-aminobenzene-1-sulphonic acid      | 3-N-ethoxyethylaminobenzene-1-sulphonic acid                         | Deep Bordeaux red        | Deep red violet          | Deep red violet          |
| 33 | 5-nitro-2-aminobenzene-1-sulphonic acid      | Oxyethylaminobenzene                                                 | Violet-brown             | Violet-brown             | Violet-brown             |

| 3  | Dyestuff                                 |                                                                          | Dyeing on leather  |                        |
|----|------------------------------------------|--------------------------------------------------------------------------|--------------------|------------------------|
|    | Diazo-component                          | Azo-component                                                            | On the surface     | In the interior        |
| 24 | 5-nitro-2-aminobenzene-1-sulphonic acid. | Dioxyethylaminobenzene.                                                  | Pure Bordeaux red. | Powerful Bordeaux red. |
| 35 | 5-nitro-2-aminobenzene-1-sulphonic acid. | 3-oxyethylamino-1-methylbenzene.                                         | Bordeaux red.      | Bordeaux red.          |
| 36 | 5-nitro-2-aminobenzene-1-sulphonic acid. | 3-dioxyethylamino-1-methylbenzene.                                       | Bordeaux red.      | Deep dark-violet.      |
| 10 | 5-nitro-2-aminobenzene-1-sulphonic acid. | 3-di-( $\beta$ : $\gamma$ -dioxy)-propylamino-1-methylbenzene.           | Pale Bordeaux red. | Bordeaux red.          |
| 37 | 5-nitro-2-aminobenzene-1-sulphonic acid. | 3-chlorodioxyethylamino-1-methylbenzene.                                 | Deep Bordeaux red. | Dark red-violet.       |
| 38 | 5-nitro-2-aminobenzene-1-sulphonic acid. | 3-chlorodi-( $\beta$ : $\gamma$ -dioxy)-propylamino-1-methylbenzene.     | Bordeaux red.      | Deep Bordeaux red.     |
| 39 | 5-nitro-2-aminobenzene-1-sulphonic acid. | 3-chloro-4-( $\beta$ : $\gamma$ -dioxy)-propylamino-1-methylbenzene.     | Violet-brown.      | Deep violet-brown.     |
| 40 | 5-nitro-2-aminobenzene-1-sulphonic acid. | 3-oxyethylamino-4-methoxy-1-methylbenzene.                               | Grey-brown.        | Grey.                  |
| 41 | 5-nitro-2-aminobenzene-1-sulphonic acid. | 3-dioxyethylamino-4-methoxy-1-methylbenzene.                             | Red-brown.         | Red-brown.             |
| 42 | 5-nitro-2-aminobenzene-1-sulphonic acid. | 3-di-( $\beta$ : $\gamma$ -dioxy)-propylamino-4-methoxy-1-methylbenzene. | Yellow-brown.      | Brown-violet.          |
| 43 | 5-nitro-2-aminobenzene-1-sulphonic acid. | 2-dioxyethylamino-1:4-dimethylbenzene.                                   |                    |                        |

5

10

15

20

25

30

35

40

45

What I claim is:—

1. A process for dyeing leather, wherein the leather is dyed with an amino-azobenzene sulphonic acid dyestuff of the following general formula:



30 wherein X<sub>1</sub> represents H or SO<sub>3</sub>H; X<sub>2</sub> represents H, NO<sub>2</sub>, Cl, CH<sub>3</sub> or OR (R being methyl, ethyl or hydroxyethyl); X<sub>3</sub> represents H, NO<sub>2</sub>, Cl or CH<sub>3</sub>; X<sub>4</sub> represents H or NO<sub>2</sub>, with the restriction that at least one of said X<sub>1</sub>, X<sub>2</sub>, X<sub>3</sub> and X<sub>4</sub> must be other than hydrogen; Y<sub>1</sub> represents H or SO<sub>3</sub>H; Y<sub>2</sub> represents H, CH<sub>3</sub>, Cl or OH; Y<sub>3</sub> represents H, CH<sub>3</sub> or OCH<sub>3</sub>; R<sub>1</sub> represents H, ethyl, hydroxyethyl or dihydroxypropyl; and R<sub>2</sub> represents hydroxyethyl or dihydroxypropyl.

40 2. A process for dyeing leather, wherein the leather is dyed with a dyestuff from diazotized 4-nitro-2-aminobenzene-1-sulphonic acid and 3-hydroxyethylamino-1-methylbenzene, having the formula:



3. A process for dyeing leather, wherein the leather is dyed with a dyestuff from diazotized 3-aminobenzene-1-sulphonic acid and di-( $\beta$ : $\gamma$ -dihydroxyethylaminobenzene, having the formula:



4. A process for dyeing leather, wherein the leather is dyed with a dyestuff from diazotized 3-aminobenzene-1-sulphonic acid and di-( $\beta$ : $\gamma$ -dihydroxyethylaminobenzene, having the formula:



EMIL SENN.